

June 5, 1928.

1,672,052

H. R. BERRY

## PROCESS FOR GAS MAKING

Filed April 5, 1928

4 Sheets-Sheet 1



Fig. 1.

INVENTOR

Harold R. Berne

BY

Crichton Clarke

ATTORNEY.

June 5, 1928.

1,672,052

H. R. BERRY

PROCESS FOR GAS MAKING

Filed April 5, 1928

4 Sheets-Sheet 2



Fig. 4



Fig. 3



Fig. 2

INVENTOR.

Harold R. Berry

BY

Crichton Clarke

ATTORNEY.

June 5, 1928.

1,672,052

H. R. BERRY

PROCESS FOR GAS MAKING

Filed April 5, 1928

4 Sheets-Sheet 3



INVENTOR.

Harold R. Berry  
Crockett Clarke

ATTORNEY.

June 5, 1928.

1,672,052

H. R. BERRY

PROCESS FOR GAS MAKING

Filed April 5, 1928

4 Sheets-Sheet 4



*Fig. 6*

INVENTOR.

*Harold R. Berry*

BY

*Crichton Clarke*

ATTORNEY.

## UNITED STATES PATENT OFFICE.

HAROLD R. BERRY, OF BROOKLYN, NEW YORK.

## PROCESS FOR GAS MAKING.

Application filed April 5, 1928. Serial No. 267,609.

The object of this invention is a process for the production of a combustible gas from carbonaceous material, for instance, such as coal; whereby volatiles are converted and enter the gas as illuminants and carbon quantities with steam enter the gas as carbon oxides and hydrogen.

The residual gas, from distilled volatiles, after tar extraction, does not constitute gascification in application of the process to coal. The process embraces the use of compound carbon in volatile fractions of carbonaceous materials to produce hydrocarbons in the gas, and use of fixed carbon of carbonaceous materials to produce carbon oxides and hydrogen in the gas.

The process includes, for instance, production of an artificial combustible gas, similar in composition to carburetted water-gas manufactured from hard coal and oil, by the use of bituminous coal, steam and heat without oil; in which operation the oil-gas components of present practice enriched water-gas are obtained from the bituminous volatile and not from oil and blue water gas components from potential coke fractions of soft coal, instead of from hard coal or coke.

The process contains provisions for coal volatiles, now combusted in the air blast period of water-gas manufacture, to be reclaimed by their conversion into enriching fractions of the gas.

The process gas is useful for heating and power generation and the flexibility of regulation which obtains with gaseous fuels, governs the use of the process gas, minimiz-

ing the problems of peaks and stand-by fires, affording immediate steam response to fresh fuel and a nearer approach to complete combustion with reduced air quantities. 40 For the purpose of showing certain distinctions of the process gas, mention follows of a number of artificial gases in common use.

1. *Blast furnace gases.*—These are by-product, blast furnace gases. They contain carbon monoxide from reactions of the furnace charge, together with combustion products of carbon dioxide and nitrogen of large proportion jointly, well over one-half the 50 gas volume. The present process provides that combustion products be exited from the operation and diverted from the gas and that carbon combustion be incident to gas-making, not smelting. 55

2. *Producer gas.*—This gas is a primary product but, like blast furnace gases, combustion products are entrained in its composition. Indiscriminate combustion of volatile and carbon fractions of the fuel by 60 air blasting, characterizes its manufacture. In production of this gas, steam is sometimes added, which somewhat changes the gas-making reactions; but in producer gas the conglomerate of all reaction resultants constitutes the highly nitrogenous, thermally 65 deficient product of only some 50% greater heat value than by-product blast furnace

gases. Among other differentiations, the present process is distinguished from producer gas practice in the disposal of combustion products outside the gas-make and

distillation of coal volatiles, without combustion air contact for their reclamation in the product gas.

3. Oil gas is obtained by the heat treatment of oil. It is a hot gas usually containing large percentages of methane and unsaturated hydrocarbons. It is used straight and also for carburetion. The process gas of this specification is obtained from coal without oil and incorporates, as part of the process, carbon reaction with steam.

4. Coal gas, as a name, is diversely applied. The distilled volatile of coal, particularly of soft coal, is coal gas, yet when coke production is the chief purpose, it is called coke-oven gas. The "town gas" of the European city is really coke-oven gas. Machines, designed to devolatize coal for procuring gas for use, with coke as a by-product, have been called gas-producers, and from this the product of the gas-producer is found referred to as producer gas. It seems logical, and for the purpose of this specification clarifying if by coal-gas be intended, not producer gas as before described, but coal volatiles, distilled by heat, applied outside the coal container; combustion products not entering the distillate. The making of gas, by the process presented, differs from coal gas, so designated. Among these differences, the process reduces heat losses due, among other things, to radiation and transmission by combusting part of the coal under treatment to satisfy distillation heat requirements, yet diverts the combustion products from the gas-make; and also uses the heat so developed for temperature elevation, incident to the carbon-steam reactions which are prescribed to occur by the process.

40 5. Water-gas.—This gas, by many regarded as the most efficient, economic and practical of all artificial gases, is the product of the carbon and steam reaction at high temperature. The ratio of the carbon oxides to each other is chiefly dependent on temperatures and these oxides with the hydrogen released in their formation, constitutes the gas which is produced by intermittent air blast and steam contact. Part of the coal charge is combusted in the blast to afford gas-making heats for the run. No reclamation of coal volatiles is practiced in water-gas manufacture, the largest operations using anthracite and coke. The water-gas, or blue gas, emanating from the generator is mixed with oil gas for enrichment and this final mixed gas product is the gas, which is a counterpart in composition to that produced by the present process without the use of low volatile fuel and oil.

Distinguishment of the present process from water-gas practice is shown in application of the process to the production of a gas similar in composition to carburetted water-

gas. As the volatile fraction of anthracite coal or coke is too small to contain an amount of carbon which equals that compounded in the illuminant fraction of customarily rich carburetted water-gas, to produce such gas, by the process presented, requires the use of carbonaceous material, of higher volatile percentage than anthracite coal or coke, for instance, bituminous coal. In explanation, suppose there is found to be by analysis two pounds of carbon more in a certain amount of coal than that found as fixed carbon. This two pounds of carbon, then, with heat, is distillable from the coal, it constituting a component of the volatiles.

75 Appearance of this carbon as pure carbon in vapor phase, under the distillate heats employed, is impossible. Such carbon occurrence is possible only if the carbon be in union with another element or elements, if it be in compound. Thus all carbon available for volatiles, is either actually or potentially, compound carbon, and no carbon is available from coal for hydrocarbon gases and gas illuminants except it be contained within the volatile fraction. The only modification of this would be through union of hydrogen and carbon, which is quite impossible, to detectable extent, in the presence of the carbon monoxide quantities present.

80 Thus the process provides for derivation of illuminants from volatiles and procurement of carbon oxides and hydrogen from fixed carbon or that precipitated by heat treatment of the volatiles.

85 Application of the process in the production of a gas, similar to carburetted water-gas, manufactured from anthracite coal, oil and steam, is had in the use of bituminous coal and steam without oil and consists in combusting part of a coal charge, which has been previously subjected to devolatilization, and using heat, produced by the combustion, to first, distill volatiles from the remainder of the coal charge and, second, to supply thermal requirements for reacting part of the hot carbon and steam into gas, and uniting these reaction products with the distillates to form the gas.

90 105 If the process gas be made from coal of a small volatile percentage and if water gas of present practice be enriched with but small oil-gas amounts, the thermal value of the product-gas is increased but little over that of the blue water gas; but, if high volatile coal, for instance bituminous coal as cited, be used in making the process gas, and large oil quantities are employed to enrich the gas of present practice, the thermal values of the gas products are high.

110 120 In this application of the process is embodied the premise that the elemental constituency of soft coal equates the composite

analysis of hard coal and oil; that the ultimate constituents of present practice carburetted water-gas, derived from low volatile fuel and oil are balanced, in kind and 5 quantity, in the elemental make up of soft coal and steam, without oil. That, as gas illuminants are hydrocarbons, composed of hydrogen and carbon, and as the direct union of hydrogen and carbon does not occur under the operative conditions provided, 10 the carbon in the coal to equation that in the illuminants of the gas, must be within the coal volatiles, the fixed carbon of the coal reacting to blue water gas components, but 15 not to enrichment quantities.

The state of occurrence of the coal volatile, however, is not agreed upon. Among the elements constituting the volatile there always are oxygen, hydrogen and carbon. In 20 what compounds these elements abide in coal, is conjecture. Emanations of volatile fractions from the same coal differ, dependent upon temperatures, time, exit rapidity and even the design of the retort, said W. 25 H. Coleman. Merely the heat needed for their extraction, seems to produce reaction and modification of distillates. Condensates may contain phenol, creosote and its mixtures, aniline, when compound nitrogen is 30 present, the carboxyl group with its assortment of fatty acids, and the whole gamut of by-product coke oven recoveries, but what native union in the raw unheated coal, subsists between the elements of the coal volatile is simply guessed at.

The oxygen may be in certain of the above compounds or in alcohols, which break up into aliphatics, through oxidations producing the above. The last happening is often 40 claimed, because, as the oxygen content of volatiles increases from around 5% to 11 or 12% (Dueffe), olefines and heavy unsaturates also increase. This explained on the theory, that oxygen, from an alcohol, 45 through other union, yields the hydrocarbons. Within the named range of oxygen increase, methane increases and hydrogen decreases.

Though identity of the compounds, constituting the volatile fraction of coal, is conjectural, and the chemical unions of the distillates vary and depart from the state of native occurrence, nevertheless, the kind and quantity of the respective elements constituting the volatile matter, as occurring in the coal or abstracted therefrom, are known and each element, in accordance with its weight, has a given heat value. Subject to the plus or minus of formation heats, 60 these elements, though compounded, yield, in combustion, this heat.

Delivery of this heat, through combustion of a gas, into which these elements enter, is their conversion into gas illuminants.

Present practice enriched blue water gases 65 vary, dependent largely upon the character and quantity of the oil used for enrichment. The process gas products likewise vary, dependent largely upon the character and amount of volatiles in the coals used. Of 70 necessity, the constituents of all and varied enriched blue water gases are not equaled in every type and variety of coal. In general a low volatile coal is the counterpart of a lean water-gas and with increase of coal volatile 75 is a correspondent increase in gas richness.

Generalization in the comparisons between hard and soft coals, oils and gases, made here, in support of the process, may be supplemented and illustratively emphasized by citation of a specific coal and a specific gas which equate each other. The references are of ready access and authentic.

The coal; elements and their weights.

Citation, Engineers Handbook, Lionel S. 85 Marks, Harvard University, Massachusetts Inst. Tech., first edition, tenth impression, McGraw-Hill Book Co., New York, London, page 600.

"Table 2. (continued).

Locality, bed, etc, or commercial name of coal, Marianna, Pittsburgh bed.

| Proximate analysis<br>"as received" |                 |              | Ultimate analysis<br>"as received" |         |          |        | B. T. U. |            |                        |
|-------------------------------------|-----------------|--------------|------------------------------------|---------|----------|--------|----------|------------|------------------------|
| Moisture                            | Volatile matter | Fixed carbon | Ash                                | Sulphur | Hydrogen | Carbon | Oxygen   | "Dry coal" | Ash- and moisture-free |
| 1.44                                | 34.61           | 57.77        | 6.18                               | 0.78    | 5.23     | 78.76  | 7.61     | 14,450     | 15,417 <sup>11</sup>   |

The above quotation is verbatim. For reference convenience, a 'complete' analysis will be shown from the above. The total carbon shown, for instance, in the ultimate is 78.76 pounds, but in the proximate only 57.77 pounds appear as fixed. Of necessity, the difference is the amount of carbon that is not fixed, but is in compound association in the coal volatiles. The 'complete' analysis is:

| COMPLETE ANALYSIS (100 POUNDS) |          |       | 115    |
|--------------------------------|----------|-------|--------|
| Moisture                       |          |       | 1.44   |
| Fixed carbon                   |          |       | 57.77  |
| Ash                            |          |       | 6.18   |
| Volatile matter                | Sulphur  | 0.78  |        |
|                                | Hydrogen | 5.23  |        |
|                                | Carbon   | 20.99 |        |
|                                | Oxygen   | 7.61  | 34.61  |
| Total                          |          |       | 100.00 |

The complete analysis is a combination of the proximate and ultimate, which shows, without computation, the composition of the 125 volatile.

Were the coal, shown in analysis, coked, practically all the moisture and volatiles

would be driven off and practically all the fixed carbon and ash would go to constitute the coke. In the volatile so driven off, is provided the raw material for the by-product coke oven and the constituents for illuminants of enriched water gas. In the potential coke is the fixed carbon reactable with steam into water gas.

Sulphur, shown in analysis, is neither fixed carbon, volatile, moisture or ash of the proximate, but, is classified in the complete analysis among the volatiles, and probably with correctness, as it vaporizes around 900° F. and is frequent in the  $\text{SO}_2$  and  $\text{H}_2\text{S}$  compounds.

In assembling the data, a standard carburetted water gas analysis follows. The gas was produced by best practice, using hard coal and oil. In citing the gas, the purpose will be, to show that every element and compound in it, illuminants and straight water gas, obtained from both the oil and hard coal used, are exactly equated in the soft coal analysis, before cited.

#### 25 GAS ANALYSIS

Kent's Handbook 1923—Tenth Edition, John Wiley & Sons, N. Y., page 899.

30 "Composition by volume, water-gas, Worcester.

|                |        |
|----------------|--------|
| Nitrogen       | 2.64   |
| Carbonic acid  | 0.14   |
| Oxygen         | 0.06   |
| Ethylene       | 11.29  |
| Propylene      | 0.00   |
| Benzole vapor  | 1.53   |
| Carbonic oxide | 28.26  |
| Marsh-Gas      | 18.88  |
| Hydrogen       | 37.20  |
|                | 100.00 |

#### Density:

|          |        |
|----------|--------|
| Theory   | 0.5825 |
| Practice | 0.5915 |

#### B. T. U. from 1 cu. ft.:

|              |       |
|--------------|-------|
| Water liquid | 650.1 |
| Water vapor  | 597.0 |

50 Flame temperature, °F. 5311.2

Average candle-power 22.06"

The above citation is verbatim. Only slight comparison is possible, with the data thus far cited. The gas analysis shows a group of gases, and certain volumetric percentage, aggregating 100. The coal analysis shows an aggregation of dissimilar things totaling in weight 100.

60 The use of common denominations is necessary for comparison. The reduction of compounds to elements and of volumes to weights is obviously necessary.

A tabulation of conversion values here em-

ployed follows, containing, also, combustion heat yields in B. T. U's.

| Volumes, 60° F., 30" | Mol. Wt.                         | Cu. ft. 1 lb. | B. T. U.                |             | 70 |
|----------------------|----------------------------------|---------------|-------------------------|-------------|----|
|                      |                                  |               | Per lb.                 | Per cu. ft. |    |
| Nitrogen             | N 14 (Atom)                      | 13.464        |                         |             |    |
| Carbonic acid        | CO <sub>2</sub> 44 (Atom)        | 8.593         |                         |             |    |
| Oxygen               | O 16 (Atom)                      | 11.816        |                         |             |    |
| Ethylene             | C <sub>2</sub> H <sub>4</sub> 28 | 13.495        | 1670                    | 75          |    |
| Benzol vapor         | C <sub>6</sub> H <sub>6</sub> 78 | (*) 4.845     | 3807.5                  |             |    |
| Carbonic oxide       | CO 28                            | 13.503        | 4,368                   | (*) 323.5   |    |
| Marsh gas (*)        | CH <sub>4</sub> 16 (Atom)        | 23.826        | 23,838                  | 1009        |    |
| Hydrogen             | H <sub>2</sub> 1 (Atom)          | (*) 188.620   | (*) 61,523              | 326.2       |    |
| Carbon (*)           | C 12 (Atom)                      |               | 14,544                  |             | 80 |
| Sulphur (*)          | S 32 (Atom)                      |               | 4,050                   |             |    |
| Moisture             | H <sub>2</sub> O 18              | 21.004        |                         |             |    |
| Air (e)              | Wt. N. 76.85; O. 23.15           | 13.059        | Vol. N. 79.09; O. 20.91 |             |    |

(\*) Hempel's Gas Analysis.

(\*) Lord and Hass.

(\*) Jules Thompson, Thermo. Inves., Favre & Silberman.

(\*) U. G. I. table of gas constants.

(\*) Langes Coal Tar and Ammonia.

(\*) No thermal value is given the ash, certain calcites may shift between carbonates and oxides and readjustments of alkaline and ferrous compounds occur, but the effect on heat will be disregarded.

(\*) Lucke, Thermodynamics at 32° F., 29.92 (Ledoux) shows 341

B. T. U. reducing to 30°—60° is 323.5.

(\*) Ganot Physics, U. G. I. tables.

(\*) Thompson, Thermo. Inv. calc.

By use of the above equivalents, the weight of each gas shown in the analysis is derived, as is also, the identity and weight of the composing elements. One thousand cubic feet of the reference gas is thus shown constituted as follows:

Kent reference gas. Volumes, 60° F., 30". Compounds reduced to elements by standard at. wts.

|                               | Cu. ft. | B. T. U. | Wt. lb. | C.     | O.     | H <sub>2</sub> | N     |
|-------------------------------|---------|----------|---------|--------|--------|----------------|-------|
| CO <sub>2</sub>               | 1.4     | 0        | .163    | .044   | .119   |                |       |
| O                             | .6      | 0        | .050    |        | .050   |                |       |
| CO                            | 282.6   | 91,421   | 20,933  | 8.972  | 11.961 |                |       |
| CH <sub>4</sub>               | 188.8   | 190,499  | 7.991   | 5.993  |        | 1.998          | 105   |
| C <sub>2</sub> H <sub>4</sub> | 112.9   | 188,543  | 8.366   | 7.171  |        | 1.195          |       |
| C <sub>6</sub> H <sub>6</sub> | 15.3    | 58,255   | 3.157   | 2.914  |        | .243           |       |
| H <sub>2</sub>                | 372.0   | 121,346  | 1.972   |        |        | 1.972          |       |
| N                             | 26.4    | 0        | 1.961   |        |        |                | 1.961 |
| Total gas                     | 1000.0  | 650,064  | 44,593  | 25,094 | 12,130 | 5,408          | 1.961 |
| Av.                           | 1       | 650      | .044    | .025   | .012   | .005           | .002  |

The respective compositions of the gas and coal samples cited, are now expressed in comparable terms.

Methane, for instance, of the gas, is expressed, not only as originally given, 188.8 cu. ft. out of 1000 cu. ft. of the total gas, but also now is shown as 7.991 pounds, of which 5.993 pounds are carbon and 1.998 pounds are hydrogen.

On the one hand is shown 100 pounds of soft coal, composed of the aggregate weight of its components, on the other hand, is 1000 cu. ft. of carburetted water gas, manufactured from hard coal and oil, now shown as the weight aggregate of its constituents, each of which gases is also shown as the total weight of its designated and constituting elements.

To equation the coal and gas, an adjustment is required, as the coal quantity chosen, weighs 100 pounds and the 1000 cu. ft. of gas weighs 44.593 pounds.

- 5 The hypothesis is that the coal volatile will contain the gas illuminants, that part of the fixed carbon of the coal will be consumed for heat requirements and part re-  
10 acted with steam into water gas. On this basis, a trial constant, for a weight balance,

has been calculated as 1.3125, which will be found to check in the coal analysis.

The purpose of the following weight balance is to show that all the elements, in their required proportions, constituting the carburetted water gas cited, and manufactured from hard coal and oil are contained in the soft coal.

15

The weight balance follows:

20

| WEIGHT BALANCE                                              |                |                   |              |                                    |                               |        |                    |           |         |        |
|-------------------------------------------------------------|----------------|-------------------|--------------|------------------------------------|-------------------------------|--------|--------------------|-----------|---------|--------|
| Analysis Carburetted Water Gas made from hard coal and oil. |                |                   |              |                                    |                               |        |                    |           |         |        |
| 5.                                                          | 1000 cu. ft.   |                   |              | 1312.5 cu. ft., Kent reference Gas |                               |        | Straight Water Gas |           |         | 6.     |
|                                                             | Kent Reference | 1923 Ed., p. 899. | 6.           | Gas Components                     | Symbol                        | Wt. %  | Wt. lb.            | Wt. lb.   | Wt. lb. |        |
| Analysis - Bituminous Coal and Steam                        | 1000 cu. ft.   | 1312.5 cu. ft.    | 1000 cu. ft. | Carbonic Acid                      | C <sub>2</sub> O <sub>2</sub> | 1.83   | .22                | .04       | .16     |        |
| 100 pounds soft coal and 28.62 pounds steam                 |                |                   |              | Oxygen                             | O                             | .78    | .067               |           | .087    |        |
| equivalent with Gas analysis                                |                |                   |              | Ethylene                           | C <sub>2</sub> H <sub>4</sub> | 146.18 | 247.442.7          | 10.98     | 1.548   | 9.412  |
| Bituminous Coal, Pittsburgh Bed, Mariana                    |                |                   |              | Methane                            | C <sub>2</sub> H <sub>6</sub> | 20.08  | (2807.6)           | 4.143     | .319    | 3.824  |
| Coal Analysis from                                          | Heat and       | 1000 cu. ft.      |              | Carbonic Oxide                     | C <sub>2</sub> O              | 370.92 | 117.90.1           | 27.47     |         |        |
| Mark's Handbook 1st Ed., p. 600                             | Waste          | O                 | C            |                                    |                               | (1000) | 260.000            |           | 11.78   | 15.69  |
| Moisture                                                    | 1.44           | 1.44              |              | Marsh-Gas                          | C <sub>2</sub> H <sub>6</sub> | 186.8  | 247.50             | 10.378    | 3.623   | 7.755  |
| Ash                                                         | 6.18           | 6.18              |              | Hydrogen                           | H <sub>2</sub>                | 372.   | 468.25             | 191.287.2 | 2.58    |        |
| Fixed Carbon                                                | 57.77          |                   |              | Nitrogen                           | N                             | 26.4   | 34.65              | 2.67      |         |        |
| Reaction heats and waste (2)                                | 29.395         |                   |              | Total                              |                               | 1000   | 1312.50            | 58.407    | 4.510   | 30.99  |
| Reacted in gas (2)                                          |                | 24.33             |              |                                    |                               |        |                    | 2.68      |         | 11.84  |
| Genesible heat volatile (b)                                 | 1.11           | 25.44             |              |                                    |                               |        |                    |           |         | 15.912 |
| Latent heat volatiles (c)                                   | .90            |                   | 3.18         |                                    |                               |        |                    |           |         | 2.87   |
| Evaporation moisture (4)                                    | .115           |                   |              |                                    |                               |        |                    |           |         |        |
| Steam external (e)                                          | 1.92           |                   |              |                                    |                               |        |                    |           |         |        |
| Volatile                                                    | 34.61          |                   | 25.44/24.33  |                                    |                               |        |                    |           |         |        |
| Oxygen                                                      |                | 7.61              |              |                                    |                               |        |                    |           |         |        |
| Carbon                                                      |                | 20.99             |              |                                    |                               |        |                    |           |         |        |
| Hydrogen                                                    |                | 5.23              |              |                                    |                               |        |                    |           |         |        |
| Sulphur                                                     | .78            | 8.41              |              |                                    |                               |        |                    |           |         |        |
| Coal total (15.)                                            | 100.00         |                   |              | Unbalanced quantities              |                               |        |                    |           |         |        |
| Steam (15.)                                                 | 28.62          |                   |              |                                    |                               |        |                    |           |         |        |
| Material, total                                             | 128.62         |                   |              |                                    |                               |        |                    |           |         |        |
| Rent and Waste                                              | 41.84          |                   |              |                                    |                               |        |                    |           |         |        |
| In Gas                                                      | 53.05/28.62    | 20.99/8.41        | 66.78        |                                    |                               |        |                    |           |         |        |
| Material, total                                             | 128.62         |                   | 128.62       |                                    |                               |        |                    |           |         |        |

On the weight balance sheet, in column 1, is shown the 1000 cu. ft. of carburetted water gas, made from hard coal and oil, as set forth in the Kent reference. Applying the constant, division 2 shows 1312.5 cu. ft. of the same gas, in which symbols and thermal values of the constituting gases are shown. To check any quantity shown in division 2, multiply the corresponding item in column 1 by the constant, 1.3125.

The weight of each of the constituting gases, shown in column 2, is segregated, in

proper ratio, to the constituting elements, and these apportioned weights are set down in either column 3 or 4, dependent upon whether the particular gas be an illuminant and derived from oil, or a constituent of blue water gas, derived from coal and steam.

35

Divisions 2, 3 and 4, show the composition of 1312.5 cu. ft. of the Kent reference gas, divisioned into respective weights of their composing elements of hydrogen, carbon and oxygen, classified appropriately as illum- 40

45

nants and straight water gas and summarized as follows:

1312.5 cu. ft., carburetted water gas manufactured from hard coal and oil.

| 5  | B. T. U. |             | Illuminants |                |       | Blue gas |                |      |
|----|----------|-------------|-------------|----------------|-------|----------|----------------|------|
|    | Total    | Per cu. ft. | C.          | H <sub>2</sub> | C     | O.       | H <sub>2</sub> | N    |
| 10 | 853,209  | 650         | 20.99       | 4.51           | 11.84 | 15.917   | 2.58           | 2.57 |

Division 5 of the weight balance.—All the coal, either hard or soft, fed into a gas generator, does not enter the gas. Heat is required to drive off the volatile of soft coal, make steam, elevate temperatures and supply reaction heat requirements. These needs are satisfied by combustion of part of the 15 coal charge. To determine the part of the coal used for heat production and the part reacted into gas, reference is again had to the Kent citation, in which appears a heat balance of a carburetted water gas operation.

20 1000 cu. ft. of the gas is shown to be a mixture of 645 cu. ft. of blue water gas and 355 cu. ft. of oil gas. 23.5 pounds of carbon, exclusive of ash and unconsumed coal, is used 25 in making the 645 cubic feet of water gas, or 36.34 (a) pounds of carbon are used in combustion and reaction to produce 1000 cu. ft. 30 of water gas,  $(\frac{23.5}{645})$ .

35 Besides the carbon actually incorporated in the gas (about 15 pounds per 1000 cu. ft.), through its combustion, certain heat requirements are satisfied. These include: The energy of the CO produced, the energy absorbed in the decomposition of the steam, the heat carried off by the escaping air blast products, the heat loss by radiation from the shells, the heat carried away from the shells

40 by convection and the sensible heat carried away with the ash and unconsumed coal.

45 In the allowance of 36.34 pounds of carbon, per 1000 cu. ft. of water gas, is included the amount of carbon required for combustion to elevate coal temperatures to reactive 50 heat. Yet, in deriving water gas illuminants from oil, the oil must be heated, and in obtaining these illuminants from the soft coal volatile, the volatile must be heated, and this heat requirement is not included in the above 55 carbon allowance. Figuring the volatile as requiring an average temperature elevation of 1000° F. for their liberation from the coal, their sp. ht. .45 and their quantity, the 60 34.61 pounds of volatile in the 100 pound coal sample cited, the heat requirement for sensible temperature elevation of the volatiles is  $(1000 \times .45 \times 34.61)$ , or 15,574 B. T. U., requiring the combustion of 1.11 (b) lbs. of coal, at 14,000 B. T. U. per pound.

65 Not only, however, must the volatiles be heated but also thermal force be supplied to break the tension which holds them within the coal.

70 On the basis of the same heat requirement, weight for weight, for production of gas from petroleum as its liberation from soft coal, this heat requirement is—

75 1      2      3  
34.61:35 as X:12,841 B. T. U.; wherein 3 is the heat rendered latent in the gasification of oil. (H. in the Kent reference), 2, the mass of 5 gallons of petroleum at 7 pounds to the gallon; 1, the weight of the coal volatile and X, the B. T. U.'s required to liberate 80 the volatiles from the soft coal. X is 12,700 B. T. U. or .90 pounds of carbon (c).

85 Though water gas steam requirements have been equationed under count "a", no allowance is made for ridding the soft coal of its moisture percentage. This factor will be 1:44 (weight of moisture in the coal sample) X

$$\left( \frac{\text{sensible latent}}{(212 - 60) + 971} \right) = 1617.12 \text{ B. T. U.} = .115 \text{ lb. C (d)}$$

90 In the steam requirement for water gas manufacture, estimated in count "a" above, the provision embraces the heat requirements of steam after it enters the generator, but does not include the heat to make the steam before it enters the apparatus.

95 The heat absorption for water at 60° F. to steam at 350° F. is 1160 B. T. U. per pound (saturated steam tables). 23.76 pounds of steam enter the composition of 1000 cu. ft. of water gas (see water gas analysis). Thus, 100 27,562 B. T. U. (1160 × 23.76) are required in

steam composition in the production of 1000 cu. ft. of gas. The heat carried off by the escaping blast products in manufacturing 1000 cu. ft. of water gas is 74,152 B. T. U. (see Kent reference). Thus, the exhaust 105 heat carried away from the generator in making 1000 cu. ft. of gas is some 20,000 B. T. U. greater than double the heat required to make the steam entering the 1000 feet of gas.

110 There are a number of simple and satisfactory devices which utilize the exhaust

heat from the generator to make all the steam used in making the gas. This, of course, entails no fuel cost for steam.

- A number of factors figure in these constructions involving heat transmission and excess steam in the gas making, but the heat surplus is so large that no particular ingenuity is required to obtain all needed steam making heats from the exhaust.
- 10 Ignoring exhaust heat economy, and figuring coal at 14,000 B. T. U. per pound and a boiler efficiency of 65%, 3 pounds of coal (e) will produce the steam required for 1000 cu. ft. of gas.

18

$$\left( \frac{1160 \times 23.6}{14,000} \times \frac{100}{65} \right)$$

For reference convenience, the above items are tabulated as follows and referred to on 20 the weight balance by the letters shown, viz:

|                                                                                                                | Carbon pounds. |
|----------------------------------------------------------------------------------------------------------------|----------------|
| (a) Amount of carbon required for use, exclusive of ash and unconsumed coal, to produce 1000 cu. ft. water gas | 36.34          |
| 25 (b) For elevating the temperature of volatiles in 100 pounds of soft coal (per coal sample)                 | 1.11           |
| (c) For heat to liberate volatiles from the above                                                              | .90            |
| (d) For moisture evaporation of 100 pounds sample coal                                                         | .115           |
| (e) For steam making ( $\frac{3 \times 640}{1000}$ )                                                           | 1.92           |
| 30 (f) For estimated loss in unconsumed coal and ash per 1000 feet of water gas make (see Kent reference)      | 9.90           |
|                                                                                                                | 50.285         |

The amount of fixed carbon in the Pittsburgh coal sample, shown in analysis, is 35 57.77 pounds. This amount of carbon seems sufficient compared with the above total, to drive off the volatiles, satisfy heat requirements, and produce some 1000 cu. ft. of water gas. The showing of a smaller gas volume, in the weight balance, is due, however, to increase of the item of waste, as a precaution against imperfect or careless operation and the unaccountable losses between theory and practice sometimes observed.

45 The coal analysis (Div. 5) is set down in vertical sequence. The quantities are distributed to 'heat and waste' or to 'gas composition' as oxygen, fixed carbon, carbon of the volatile and hydrogen. The steam quantity entering the gas, is shown horizontally from the fixed carbon figures of the coal analysis, under caption 6.

Below the gas distribution shown in divisions 1, 2, 3 and 4 is incorporated an additional 55 640 cu. ft. of gas composed of the familiar products of the water gas reaction. After satisfaction, through combustion, of the thermal requirements placed upon the fixed carbon of the coal, the residue carbon, 60 with the steam quantities shown, constitutes this additional 640 cu. ft. Hard coal with oil is shown in balance with soft coal without oil; the determinations being derived from authentic analyses.

65 Without noting the small nitrogen quan-

tity, valueless in combustion, the gas of 1953 cu. ft. is in complete weight balance with the 100 pound coal sample plus 28.62 pounds of steam.

1. The total weight of the carbon in the 70 volatile fraction of the coal is 20.99 pounds; the weight of carbon in the illuminant fraction of the gas is 20.99 pounds.

2. The remainder of the carbon in the 75 coal is the fixed carbon, 57.77 pounds. Part of this carbon is shown either wasted or combusted, for purposes before described and referred to by letters on the weight balance, thus:

|     |               |
|-----|---------------|
| (f) | 29.395 pounds |
| (b) | 1.11 "        |
| (c) | .90 "         |
| (d) | .115 "        |
| (e) | 1.92 "        |

80

85

Total 33.44 pounds of fixed carbon combusted or wasted in the gas making, leaving 24.33 pounds of the fixed carbon of the coal available for reaction into water 90 gas constituents. The total amount of carbon in the non-illuminant part of the gas is 24.33 pounds.

3. The steam quantity, 28.62 pounds, is distributed in proper ratio, to hydrogen, 95 3.18 pounds, and oxygen 25.44 pounds. To this oxygen quantity, provided by the steam, as added the 7.61 pounds of oxygen in the coal, making 33.05 pounds of oxygen in the steam and coal supplied. The total oxygen 100 content of the gas is 33.05 pounds.

4. When the oxygen of the steam thus joined the carbon of the coal, of necessity, the 3.18 pounds of hydrogen in the steam was released; adding to this the 5.23 pounds of hydrogen in the coal, makes 8.41 pounds. In the gas, its illuminants and, in free state, are 3.90 pounds, totaling 8.41 pounds of hydrogen in the total 110 gas, exactly the same as that contained in the steam and coal supplied.

5. Needless to say, the illuminants and blue water gas constituents of the weight balance equal the total gas in volume, weight, distributed elemental weights and 115 thermal value.

6. The total raw material is coal 100 pounds, steam 28.62 pounds, totaling 128.62 pounds. To waste and combustion is charged 120 41.84 lbs., leaving a net weight for reaction quantities of 86.78 lbs. The total weight of the gas is 86.78 lbs.

The weight balance certainly substantiates the statement, that all the elements, and the needed quantity of each, composing a carburetted water gas, produced from hard coal and oil, are fully contained and equated in soft coal and steam and no oil, including also satisfaction of all thermal requirements incident to the gas manufacture.

125

130

The weight balance is complete and its summary is this:

| Materials     | To waste    | To heat  | To gas         |       |      | The gas                             |           |             |              |
|---------------|-------------|----------|----------------|-------|------|-------------------------------------|-----------|-------------|--------------|
|               |             |          | H <sub>2</sub> | C     | O    | Wt.                                 | Cu. Ft.   | B. T. U.    |              |
| Coal.....     | 100.00 lb.  |          |                |       |      | CO <sub>2</sub> .....               | 1.54 lb.  | 12.33       |              |
| Moisture..... |             | 1.44 lb. |                |       |      | O.....                              | .067      | .79         |              |
| Ash.....      |             | 6.18     |                |       |      | C <sub>2</sub> H <sub>4</sub> ..... | 10.98     | 148.18      | 247,482.7    |
| Fixed C.....  |             |          | 33.44          |       |      | C <sub>6</sub> H <sub>6</sub> ..... | 4.143     | 20.08       | 76,459.7     |
| Oxygen.....   |             |          |                | 24.33 |      | CO.....                             | 55.773    | 752.92      | 243,667      |
| Vol. C.....   |             |          |                | 20.99 |      | CH <sub>4</sub> .....               | 10.378    | 247.80      | 260,030      |
| Hydrogen..... |             |          |                | 5.23  |      | H <sub>2</sub> .....                | 3.90      | 736.41      | 240,217.2    |
| Steam.....    | 28.62       |          |                |       |      | N.....                              | (2.57)    | 34.65       |              |
| Hydrogen..... |             |          |                |       |      | Wt. ....                            | 86.78 lb. | 1,953       | 1,057,736    |
| Oxygen.....   |             |          |                |       |      | Waste. ....                         | 8.40 lb.  |             |              |
| Material..... | 128.62 lbs. |          | 8.40           | 33.44 | 8.41 | Heat. ....                          | 33.44 lb. |             |              |
|               |             |          |                |       |      | Gas. ....                           | 128.62    | 1,953 c. f. | per cu. ft.  |
|               |             |          |                |       |      |                                     |           |             | 540 B. T. U. |

The cost of the gas for labor and material, based upon soft coal at \$2.00 per short ton, double shift labor and a daily production of 5000 M. cu. ft. of gas daily is:

| Gas<br>cu. ft. | Coal             |         | Labor<br>cost | B. T. U.        | Cost<br>labor and<br>material |
|----------------|------------------|---------|---------------|-----------------|-------------------------------|
|                | Wt.              | Cost    |               |                 |                               |
| 1953           | 100 lb.....      | \$0.10  |               | 1,057,736       |                               |
| 5000 M.        | 128 sh. ton..... | 256,000 | \$30.00       | Per cu. ft. 540 | \$280.00                      |
| 1000           | 51.2 lb.....     | .0512   | .006          | 540,000         | .0572                         |
| 39000          | 1 sh. ton.....   | 2.00    | .234          | 21,000,000      | 2.234                         |

15 Description of apparatus and its functions.

In the accompanying drawings, there is shown an assembled twin-unit apparatus and enlargements of certain of its parts, constituting a mechanism and method for a continuous operation of the process presented. There is, also, shown an apparatus operable intermittently by the subject process.

20 Any departure from the apparatuses as shown, which permits the functioning or operation of the process disclosed, is within the claims of the invention. The accompanying drawings are but illustrations of the application of the process to operation, and the many designs, types and variations of construction by which the process may be operable are within the scope of the specification and claims hereof.

25 In the accompanying drawings, like reference numerals indicate corresponding parts in the different figures of the drawings. Fig. 1, in vertical cross section and graphic, shows two similar generators of cylindrical design constituting an apparatus operable by the process described in this specification.

30 Fig. 2, is a top view of either of the similar generators shown in Fig. 1.

35 Fig. 3, and Fig. 4, are enlargements of two certain parts of Fig. 1.

40 Fig. 5, shows certain pattern derivations, and

45 Fig. 6 shows in vertical section a generator, applicable for intermittent operation of the process.

In Fig. 1 (a) represents the outer of two 50 hollow shells of a gas generator; (b) the inner shell; (c) indicates insulation material attached to the inner surface of the hollow shell (b), Fig. 1; (d) is a fire grate; (e) is an air blast line with a valve located 55 therein; (f) is an exit gas line with a valve therein, indicated; (g) is a smoke stack with a cut-off valve indicated, to which is joined four tributary smoke pipes, indifferently 60 designated (gt); (h) shows the cross-section of a large washer-like ring, which rests atop the outer and inner shells (a) and (b), Fig. 1, to the top rim of each of which shells it is firmly attached; (i) is a conic section, the 65 large circumference of which, evenly abuts all around the small circumference of (h), Fig. 1, to which it is firmly attached on the down sides of both places; (j) represents, generally, a number of rod braces, attached 70 at one end to the undersurface of (i) Fig. 1, and the inner surface of hollow shell (b) Fig. 1. Thus far in the assemblage, the outer concentric shells now support a plain 75 circular ring-like sheet, firmly attached to their respective top rims, which circular sheet at its inner circumference unites with a collar-like conic sloping downward and toward the general center; the conic being strengthened by rod braces from its lower surface to the inner surface of the inner-most of the two shells.

The inner surface of insulating material 80 forms a circular well strongly supported with a beveled opening at its top. Conics (k) and (z), Fig. 1, are firmly united by angle iron at their concentric circumferences and the unit formed by the union of the two pieces rests upon, but is not attached to the beveled sides (i) Fig. 1 of the opening into the interior well. Four circular openings 85 are provided in (k) Fig. 1, carried with angle-irons to accommodate branch-flues, (gt), Fig. 1.

A top for the insulated well is formed 90 by a heavy circular sheet, (m) Fig. 1, to the circumference of which is securely attached

by angle-iron the larger circumference of the conic (n) Fig. 1, which conic is braced by a number of rod supports, (o), Fig. 1, to the interior side of the lid or cover, (m) Fig. 1. In Fig. 1 the cover is shown in place; its beveled edge (n) Fig. 1 resting upon and concentric with the conic (k) Fig. 1, and conic (k) Fig. 1 resting upon the bevel of the well opening (i) Fig. 1. A series of grappling rings (p) Fig. 1 are attached to the top structure by which it may be put in place or lifted by the plant crane. The top plate, (m) Fig. 1, has four elliptical holes, collared with angle-irons to accommodate the tributary stacks (gt), Fig. 1.

The top plate (m) Fig. 1 has a circular opening at its center (r) Fig. 1, affording communication with the interior of main stack (g) Fig. 1. A casting (s) Fig. 1 surrounds this central hole, (r) Fig. 1 and supports stack (g) Fig. 1; (t) and (w) Fig. 1 are coal hoppers, equipped with sliding traps at the bottom and lids at the top. A pipe (x) Fig. 1, enters the interior of the unit shown in Fig. 1, through its top as does also pipe (y) Fig. 1.

The remaining interior structure is the piece formed, by union at their larger circumferences, of the two conics (aa) and (bb) Fig. 1, the smaller of these being supported at its small circumference by angle-iron to the undersurface of the top plate (m) Fig. 1. The space bounded by the interior surfaces of the piece composed of conics (aa) and (bb) will be referred to as (A), Fig. 1; the irregular circular space bounded by the outside surface of this piece and the inner surfaces of (l), (k) and (m), Fig. 1 will be referred to as (B) Fig. 1; and the space bounded by the interior surface of the insulation (c) Fig. 1, and the outside surfaces of (l) and (k), Fig. 1 is designated (C), Fig. 1.

Situated to the right of the unit described, is a second similar unit, corresponding parts of which are symbolized the same as in the unit shown to the left with the addition of a (').

Fig. 2 is a top view of either unit shown in Fig. 1, with corresponding lettering of parts, as an aid to the description of Fig. 1.

Fig. 3 is an enlargement of that part of the left hand unit of Fig. 1 indicated by the lettering. On this figure, because of its enlargement, are shown lugs (4<sup>a</sup>) and (4<sup>b</sup>), Figs. 1, 2 and 3, typical of a series attached firmly to respectively the top, (m) Figs. 1, 2 and 3, and to the rim (b) Figs. 1 and 3, by which pins, (4<sup>c</sup>), Figs. 1, 2 and 3, may firmly hold in place the assemblage of the top of the apparatus, in the manner shown, and yet, by their removal with the stroke of a hammer, permit the entire top arrangement to be lifted by use of a crane and the loops (p) Fig. 2.

Fig. 4 is an enlargement of that part of the left hand unit of Fig. 1 indicated by the lettering. Without reference letters, a sliding pipe section with collar, is shown in the tributary flue (gt) Figs. 1 and 4, which enables severance of the flue structure when the lid of the apparatus is to be lifted.

Fig. 5 is a sample cutting room pattern, fully indicative, without comment, of the general method for laying out the conics.

Fig. 6 is a rough cross-section design of an apparatus, operable by the process with intermittent cycle, which is shown with sufficient detail without reference symbols to answer the purposes of the specification.

Use of the process disclosed, in a twin generator operation, is illustrated in the drawings, Fig. 1, with elaborations as shown in Figs. 2, 3, 4 and 5.

The apparatus is not shown as the best adaptation of the process, nor is a perfect functioning of the process claimed for the mechanism. The twin set shown in the drawings is presented as one of any number of constructions, which may incorporate in its operation the tenets of the subject process, all mechanisms so functioning being within the claims hereof.

In operation, when coal is the fuel used, to coal the two units (Fig. 1) the coal is fed through hoppers (t) and (w), and (t') and (w'), Fig. 1. The fuel passes downward through spaces B and B' (Fig. 1), to the grates of the respective units, (d) and (d') Fig. 1. After the grates are filled, conforming with the declivity angle, the feed rises upon itself until the entire spaces, indicated as B and B' (Fig. 1) are filled. When this occurs the traps in the bottoms of the respective hoppers are closed. Each hopper is filled for later replenishment of the interior fuel magazine, shown as the coal filled region of the right-hand unit Fig. 1, and its top is closed. Both units are then fired and air blasted, valves in pipes (e) and (g) and (e') and (g') Fig. 1 being open, all other valves closed.

The first unit to attain reactively high temperature in its first bed located upon its respective grate (d) or (d') Fig. 1, is put on a steam run to generate water gas, the other remaining on air blast.

To inaugurate the water gas run, stack and blast valves are closed, and the steam and the gas lines opened. In the right hand unit of Fig. 1, for instance, the valves on pipes (e') and (g') are closed and y' and f' are opened. The valve on the pipe shown in Fig. 1, as X and its continuation as x' is opened. The reciprocal twin-unit operation is on. The unit shown to the left in Fig. 1 is on air blast, the unit shown to the right in Fig. 1 is on water gas-making run.

The path of the combustion products within the unit on air blast is not that shown as

occupied by coal in Fig. 1. Through this region B and B' of the respective units, pass the four tributary flues designated as (gt) and (gt') in the respective figures, but no access is provided. The combustion products of the unit in blast, Fig. 1, rise to the central stack (g), through the space A and through space C to and through the tributary stacks (gt). The hot combustion products pass, not through the fuel atop the fire-bed in space B, but around it through space C and within it, through space A and without contact. The fuel in the fire-bed is burned. The fuel above the fire-bed is heated. The rising temperature of the fuel, above the fire-bed, in the magazine, space B, in the drawing, produces coke and distillation of the volatiles in the coal, and its partial or complete reduction to coke. The exit for such distillates is provided through pipe (x and x', Fig. 1). As fuel in the fire-bed is consumed, it is automatically and continuously replaced with fuel, wholly or partly devolatilized to coke, from the magazine; and replenishment of the magazine occurs, from time to time by pulling the lever and sliding the trap in the bottom of a coal hopper, which is again refilled when the trap is closed.

The volatiles driven off from the magazine coal of the unit on air blast, have been carried over and delivered into the fuel magazine of the unit in gas-making run. In the gas-making run the steam line (Y') Fig. 1 is delivering the steam requirement of the run into the magazine of the unit in run. Thus, the steam, so delivered, and the volatiles from the twin unit on air blast, augmented by distillates from the unit in gas-making run journey downward through the magazine coal and increasing temperatures, through space B' Fig. 1, upon the fire-bed atop grate (d') Fig. 1, through and among the incandescent carbon and, reacted, exit through the gas-line (f') Fig. 1.

For a piece of fuel to reach the fire-bed it must journey from the hopper traps, down the entire vertical length of the magazine. In the journey, it will experience repeated blasts and attain high temperature and devolatilization. The original fuel, having lost much of its volatile fraction, in its downward journey through the fuel magazine, reaches the fire-bed where, excepting for unconsumed quantities, its carbon is either reacted through combustion, to dioxide and heat production or to monoxide and gas production, dependent upon which cycle phase governs when it is reacted. It matters little to which reaction the carbon responds, as the heat balance is the same in either case.

Vaporized volatiles are constantly enroute from the unit on air blast to the one making gas.

Potential coke of the fuel, is constantly consumed; first, in combustion, to produce heat with which to distill coal volatiles and with which to produce the gas-making reactions, and, second, the reaction with steam, by which gas is produced consisting of oxides of the carbon and hydrogen released from the steam.

The process provides that part of the carbon of a fuel charge shall be combusted to furnish heat to drive off volatiles and elevate temperatures for the reaction of another part of the carbon with steam into its products. Also the process provides for non-entrainment of combustion products and a gas composition into which the coal volatiles, fixed carbon and steam are reacted.

Combustion products that may evade the exit draughts, through the main and tributary stacks, are carried over by the apparatus arrangement shown, into the unit on gas-making run, where carbon dioxide is reacted with carbon into carbon monoxide ( $\text{CO}_2 + \text{C} \rightarrow 2\text{CO}$ ). The sensible heat of the carbon dioxide is saved and the thermal cost for the conversion is confined to heat absorption. Also, the volume of the resulting carbon monoxide is double that of the introduced carbon dioxide.

Any carbon deposited from vapor phase or other cracking, eventually arrives in the fire-bed, where its thermal value is reclaimed either through combustion and heat production or through reaction and gas production. Heavy distillates from the fuel volatiles may so increase their hydrogen percentages and lower their boiling points, within the meaning of the process.

The scope of the process extends to and includes the use of any carbonaceous materials which will respond to the treatment prescribed by the process.

Excepting for, 1st, the sensible heat carried outside the apparatus by air blast products, which is reduced by heat absorption of the magazine coal, and, 2nd, apparatus radiation, also reduced by the double shell construction, and, 3rd, the sensible heat carried away by the ash and unconsumed fuel, and, 4th, the sensible heat of the gas product as delivered into the gas line, and, 5th, the potential heat yield of uncombusted carbon in the ash, excepting for these items and with their deduction, it is inconceivable how any of the heat value of the coal can do aught but appear in the gas. There is no other exit. It is just this conversion of both the coal volatile and its fixed carbon, with exclusion from the gas of combustion products, which constitutes the essence of the process. In this, let it be mentioned, that thermal values are as indestructible as matter and that a heat balance is as true as a weight balance.

Concerning the twin set apparatus: 130

1. Installation of appropriately located steam purge jets are advisable in any apparatus construction.

5 In the twin set of the drawings, such jets (not shown) may be placed toward the top of spaces C and C', Fig. 1.

10 After the gas-making run a quick steam delivery from this location drives the gas from the space indicated, to and through the fuel-bed; so that, with inauguration of the blast, it is steam, not gas, or its combustion products, which exit through the tributary flues.

15 2. The varied composition and physical conditions as to size, regularity, etc., of the fuel, may necessitate, for good operation, mechanical changes of apparatuses. For instance, in the twin generator set shown in the drawing, the presence of slack, irregularities and mixtures of fuel sizes may make it advisable, for better operation, to deliver the distillates into the spaces A or C, Fig. 1 and into A' or C' Fig. 2, instead of into spaces B and B', Figs. 1 and 2. Such, or 20 similar changes in operation would not constitute a departure from the process.

3. Steam for reaction purposes may be delivered into the generators, at any point, other than that indicated in the drawings, 30 without departure from the process.

35 4. Though heat absorption by the fuel contained in the fuel magazines, reduces the temperatures of the conic boundary walls of the zones; nevertheless, an edging of carbon-rundum or other suitable material at the bottom edges of these conics, where they contact the firebed, will prolong the life of the interior structure of the generators.

5. In illustrating operation of the process with the twin units shown in the drawing, it was not necessary, for the purpose, to show doors in the shells, affording access to the interior of the generators. Such door may be installed at any suitable location.

45 6. Most standard shells are so equipped without specification.

55 6. Though the customary thermal debit has been made for drying the coal cited, the moisture fraction of the coal, in reality, will pass during blast from the magazine containing it, into the gas-making run of the twin generator and there be reacted with carbon into gas.

7. Operation difficulties of present carburetted water-gas practice, necessitating periodic shut-downs, due to carbon accumulations in the carburettor and super-heater are avoided by use of the process. Any such deposits eventuate in the fire-bed and are combusted or reacted without operation interruption.

8. Steam reacts with carbon, at nearly a thousand degrees below the temperature of some 2000° F. employed by best practice for the reaction. At sufficiently low tem-

peratures, however, the carbon monoxide percentage becomes as small as a few per cent and carbon dioxide increases in proportion. But, the same weight of carbon reacted to carbon dioxide, releases just double the quantity of hydrogen as it would, were the reaction to carbon monoxide. And, at the temperatures of the process firebed, around and above 2000° F., carbon dioxide reacts with carbon to carbon monoxide, in a quantity double that of the dioxide. This is mentioned in connection with the increasing temperatures encountered by the steam, in carbon contact, on its downward journey through the fuel magazines, as provided in the twin-set apparatus described.

9. Excepting the hoppers, insulating material and foundations, the twin generators are made from standard stock sizes of sheet, plate, angle-irons, rods, bolts, rivets and casting (S) Fig. 1. Dismantlement is accomplished by removing the entire flue structure, main and tributary pipes with one lift. Disengagement of the pins (4") Figs. 1, 2, 3 and 4, releases the entire cover structure, which with a single hoist is removable with the conics attached to its under surface.

10. The twin-set functions as a continuous operation with automatic fuel feed.

11. It is not claimed in operation of the process that any apparatus will drive off all possible volatiles of the coal nor completely exclude from the gas all products of combustion. The process includes the normal departures from perfect operation incident to any operation.

12. Heat absorbed for evaporation of the moisture in the coal is reclaimed, as the water vapor is carried over to the unit in gas-making run, where it is reacted with carbon, along with the supplied steam quantities.

13. It is to be noted that in delivering reaction steam into the magazine, on its journey downward, its reaction with carbon is possible, with the increasing temperatures, before it reaches the fire-bed proper. Fuel whose carbon is so reached has not completed its total heat treatment for devolatilization.

14. Adopting the quantities earlier shown in the weight balance as the operating efficiency of the twin set, there results:

The thermal value of the coal, shown in analysis, is 14,450 B. T. U. per pound, or 1,445,000 B. T. U. in the 100 pound sample, the gasification of which, produced 1953 cu. ft. of 540 B. T. U. gas, or 1,057,736 B. T. U. in total. Thus the mechanism shown, becomes a heat machine of 73% efficiency,

$$\frac{(1,057,736)}{1,445,000}$$

Forstall, in Kent, rates the carburetted water gas operation at 61%.

Estimating hard coal or coke at \$8.50 per ton, oil at 6¢ per gallon of 7 lbs. and soft coal at \$2.00 per ton, an economic efficiency of about 5 to 1 favors a bituminous coal operation in accordance with the process cited here, as against present carburetted water gas practice.

10 Fig. 7 of the drawings is a sketch of an apparatus intermittently operable by the process. It is illustratively shown as an indication of the variety of methods and apparatuses by which the process may be applied. No reference symbols are employed, as the operation is quite apparent.

The cycle of the single unit is air blow and steam run. The course of the blast is indicated through the fuel and the combustion products are shown to exit through the stack.

Distillates, produced during the air blast, may be conveyed through the pipe, leading from the top of the generator to a relief holder, not shown, and returned, through the same pipe, to the generator during the gas-making run; or they may be passed through a condenser or dephlegmator, as shown. In the latter case the fixed gases 25 may be permanently withdrawn from the apparatus for purification and use and such condensates as desired, alone, returned to the apparatus. Taps are indicated, as a method for withdrawal of any desired fractions. 30 The unit may be united for continuous operation with another generator of like or dissimilar construction, it being within the scope of the process to utilize any method of operation or mechanical arrangement, 35 which permits the process to function.

It is within the scope of the process to provide for introducing reaction steam for the gas making run through the same inlet as that which admits air quantities during 40 the blast and to provide a common exit for reaction gas quantities and combustion products, conducting them through their separate and respective channels outside the generator.

45 The originality of this invention lies in new combinations of things known, which encompasses process novelty.

A new product may be discovered or a new method for obtaining an old product, 50 but the process for doing these things must be expressed in known quantities to function. In a sense, the process gas is producer gas, excepting that combustion products are diverted from the gas-make; it is coal gas 55 excepting that potential coke is reacted to combustible gas; it is water gas, excepting that devolatilization supplants carburett-

60 By the process, depleted, nitrogenous, thermally weak producer gas is replaced by 65 a hot gas of carburetted water-gas constit-

uency; coke, tar and gas characterizing coal gas products, become hydrogen, monoxide and illuminants, and the use of hard coal or coke and oil in producing water gas is supplanted by the use of soft coal and steam 70 without oil, and the functions of carburettor and superheater of water gas practice, are performed within the magazine and relatively hot carbon of the process reaction zone.

75 In general concerning the process;



80

One pound of carbon, plus heat, combines with one and one-half pounds of water to make two and one-third pounds of carbon monoxide and one-sixth pound of hydrogen.

If hydrogen be given a thermal value of 61,523 B. T. U. per pound, and carbon monoxide, a value of 4,368 B. T. U. per pound, the products above yield in combustion 21,446 B. T. U.

$$\frac{61,523}{6} + (2\frac{1}{3} \times 4,368).$$

90

If carbon has a thermal value of 14,544 B. T. U. per pound and water has no thermal value, there is a difference in heat content of some 7,000 B. T. U.'s between the quantities reacted and the products resulting. The thermal difference is equated by the other quantity introduced,—which is heat. Carbon and water do not make hydrogen and carbon monoxide, but with the proper heat supplied, they do. Neither is mere temperature elevation the equation. The 7,000 B. T. U. thermal gain between reaction products and quantities reacted, is just exactly 100 how much cooler the fire bed is because of the reaction. 7,000 B. T. U.'s of sensible heat have become 7,000 B. T. U.'s of latent heat, reconvertible again by combustion of the product gases.

110 High temperature reactive contact strives for equilibrium through heat absorption and the conversion of sensible heats into latent heats.  $CO_2$  plus sufficient heat and carbon is 200; acetylene + water + enough heat, is 115 methane plus carbon monoxide,



Oxygen abandons its hydrogen for carbon union, thermal value and the conversion of 120 sensible heat intensities to latency by heat absorption. The remaining carbon saturates to methane in equilibrial accommodation.

The most important agencies functioning 125 in these heat conversions are the great combustion products, water and carbon dioxide.

The process presented is that of establishing, by combustion, intense sensible heat within a carbonaceous material, which heat 130

is made available for use outside and away from the material, by its absorption and conversion to latency through the production of gaseous reaction products, the thermal value of which is augmented by entrainment of volatile heat values and exclusion of thermally valueless combustion products and in this combination is the process claim for novelty.

10 Any carbonaceous materials which severally, or in combination, or in combination with other materials may be used in operation of the process are included within its scope, including such physical states as 15 solids, semi-solids, liquids and combinations of these.

10 It will be seen that the present process serves, in effect, to maintain a combustion zone and a coking zone both supplied with 20 carbonaceous fuel, the coking zone being above and in gravity communication with the combustion zone. In operating the twin process, there are, of course, two combustion zones and two coking zones. The process 25 may be so operated as to produce any desired degree of coking of the solid fuel.

What is claimed as new is:

1. A process for manufacturing a heating and illuminating gas, which consists in combusting part of a quantity of solid fuel by air blasting and diverting products of such combustion outside and away from the combustion zone, and during such combustion period distilling volatiles out of and away 35 from solid fuel superimposed upon the burning fuel, and when a desired incandescent heat is attained therein discontinuing such combustion, and then delivering into incandescent fuel steam and volatiles distilled 40 from solid fuel, thereby producing, enriching and fixing a combustible gas.

2. A process for manufacturing a combustible gas, which consists in establishing a plurality of incandescent beds of solid fuel, in at least one of which beds combustion with air is in progress, and in another fuel bed carbon and steam are being reacted to water gas, and distilling volatiles from the solid fuel superimposed upon the bed which 50 is in combustion, and conducting such distillates away from the fuel from which they are distilled, and delivering them, mixed with steam, into another of the incandescent beds of solid fuel in which water gas is being produced by the reaction of steam and fuel, and from which combustion products of air and fuel are excluded, and thereby forming a combustible gas.

3. A continuous process for manufacturing a heating and illuminating gas, preferably from any high volatile fuel, which consists in establishing two incandescent solid fuel beds, each having a distillation bed of solid fuel resting thereon, delivering air into the first such bed, and producing combustion

of a part of the fuel thereby, excluding air from the second such incandescent fuel bed, distilling volatiles from the distillation bed atop the first fuel bed by heat delivered thereinto from the hot combustion gases 70 emanating from the first fuel bed, delivering volatiles so distilled and steam into the second incandescent fuel bed to make, enrich and fix a water gas from which combustion products resulting from the reaction of carbon and air are substantially excluded, and in reversing the operation by excluding air from the first incandescent solid fuel bed, delivering air to the second such fuel bed, distilling volatiles in like manner 80 as before from the distillation bed of solid fuel atop the second bed of incandescent solid fuel, delivering volatiles so derived and steam into the first incandescent solid fuel bed, whereby alternately one or the other of the two solid fuel beds is in combustion with air supplied, and the other with air excluded, is producing the gas composed of the constituents of water gas from the reaction of steam and carbon and illuminants derived from volatiles distilled from the solid fuel without material dilution with any substantial amount of combustion products resulting from the combustion of the fuel.

4. A process for producing combustible gas which consists, in incandescing one solid carbonaceous bed, withdrawing products of combustion therefrom while simultaneously utilizing their heat to distill volatiles from a second carbonaceous bed, delivering distilled volatiles, with their entrained heat, and with steam to a third solid carbonaceous bed of partially devolatilized solid fuel in incandescent state, the latter bed serving, with steam and volatiles supplied thereto, 100 to make, enrich and fix water gas.

5. A process for producing a combustible gas, which consists in establishing two separate incandescent beds of solid fuel into one of which air is introduced and combustion is 110 in progress, and in the other air is excluded and steam is introduced and the production of water gas is in progress, and distilling volatiles from solid fuel superimposed upon the fuel in combustion, and delivering such distillates and steam into the fuel being reacted into water gas, whereby water gas is produced and enriched, and combustion products are substantially excluded therefrom.

6. A process of producing combustible gas, which consists in maintaining two combustion and two coking zones all supplied with solid carbonaceous fuel, each coking zone being above and in gravity-communication with one of the combustion zones, each of which combustion zones is in a state of incandescence, and, establishing combustion in the first combustion zone with air, withdrawing resultant combustion produc- 125 130

therefrom, utilizing heat of said first combustion zone and of said combustion products to distill volatiles from solid fuel in the first coking zone, conducting volatiles so derived with entrained heat and steam into and through the body of fuel in the second coking zone, said steam and volatiles, together with any additional volatiles derived in the second coking zone being conducted into contact with incandescent solid fuel in the second combustion zone to produce, enrich and fix a combustible water gas.

7. A process for manufacturing a combustible gas, which consists in alternately subjecting a solid fuel mass, first to combustion with air, and second to water gas production by reaction with steam, there being superimposed upon such fuel mass a quantity of solid carbonaceous fuel, and while combusting the fuel mass with air distilling volatiles from the superimposed solid fuel, and while reacting the fuel mass with steam into water gas delivering thereinto volatiles distilled from solid carbonaceous fuel, whereby an enriched water gas is produced without substantial entrainment of combustion products produced from the combustion of the fuel and air.

8. A process of making combustible gas in twin gas generators, each generator having a gas generating solid fuel bed and a solid bituminous fuel distillation zone, which consists in air blasting a gas generating fuel bed to incandescence, distilling the bituminous fuel in a distillation zone, by passing the air blast gases therearound, passing products of said distillation from one distillation zone to the distillation zone in the second unit and mixing steam with said products prior to entering the gas generating zone of the second unit, and

9. A process of making combustible gas in a generator having a solid fuel bed and a solid bituminous fuel distillation zone which consists, in air-blasting the gas generating solid fuel bed to incandescence, distilling solid bituminous fuel in the distillation zone by heat from the air blast gases, passing products of said distillation outside

of the distillation zone from which they are distilled, then passing distillation products into and through a distillation zone, and mixing steam with said products prior to entering the gas generating zone and after entering the distillation zone, and then generating combustible gas by passing the mixed steam and distillation products through said gas generating zone.

10. A process for producing a combustible gas, which consists in producing water gas from any solid fuel by intermittent air blast and steam contact, and during the air blast period diverting away the products of combustion with air, and distilling volatiles from solid fuel which is in contact with the incandescent fuel bed, and during the period of steam contact delivering with the steam, distillates from solid fuel for reaction with the steam in the incandescent fuel bed whereby an enriched water gas is produced substantially free from combustion products from the reaction of air and fuel.

11. A process for producing a combustible gas from solid carbonaceous materials of the higher volatile classification, which consists in reacting carbon of such materials and steam into water gas by alternate air blast and steam contact, and distilling, and removing from combustion by the air blast, volatiles from such materials during the air blast period with heat produced thereby, and contacting volatiles derived in such manner and steam with carbon of such materials rendered incandescent by air blast, whereby a combustible gas of enriched water gas constituency is produced, substantially free from the combustion products of air blasting.

12. A process for producing a combustible gas, which consists in incandescing by air blast, one of two solid fuel beds and with heat so produced distilling volatiles from the solid fuel of the second bed and conducting volatiles so produced away from the combustion zone of the first bed, and discontinuing the air blast into the first bed and with air excluded delivering steam and volatiles distilled from solid fuel into the said first fuel bed whereby a combustible gas is produced.

HAROLD R. BERRY.